# EUROPEAN PATENT SPECIFICATION

(11) **EP 0 875 317 B1**
(45) Date of publication and mention of the grant of the patent: **21.08.2002**
(21) Application number: 98107552.6
(22) Date of filing: 24.04.1998
(51) Int. Cl.: B22D 11/14, B22D 11/00

(54) **Method and apparatus for casting metal wires, bars and tubes in an upwardly direction**
Verfahren und Vorrichtung zum Giessen von metallischen Drähten, Röhren und Metallsträngen von unten nach oben
Procédé et dispositif pour la coulée de fils, tubes et barres métalliques dans une direction ascendante

(30) Priority: 29.04.1997 FI 971818
(43) Date of publication of application: 04.11.1998
(73) Proprietor: Outokumpu Oyj, 02200 Espoo (FI)
(72) Inventor: Koivisto, Markku, 28330 Pori (FI)
(74) Representative: Zipse + Habersack

(56) References cited:
- EP-A- 0 165 456
- EP-A- 0 481 380
- FR-A- 1 489 021
- FR-A- 2 367 560
- US-A- 3 746 077
- PATENT ABSTRACTS OF JAPAN vol. 008, no. 028 (M-274), 7 February 1984 & JP 58 187243 A (ATSUMI OONO), 1 November 1983
- PATENT ABSTRACTS OF JAPAN vol. 009, no. 098 (M-375), 27 April 1985 & JP 59 223144 A (SUMITOMO KINZOKU KOGYO KK), 14 December 1984

## Description

The present invention relates to a method and apparatus whereby particularly non-ferrous metal wires, bars and tubes are cast continuously in an upwardly orientation, but the casting is not carried out directly vertically, but in a somewhat inclined direction upwards. After a primary cooler, the cooling of the product takes place as direct water cooling.

The conventional vertical casting method is a method where the wire, bar or tube is cast vertically upwards, and the equipment consists of a primary cooler connected to the casting nozzle as well as of a secondary cooler. When casting for instance a wire with a diameter of 8 mm, which is the most common diameter in cast copper wires, the total length of the coolers is roughly of the order of 2 m. The crystallization and primary cooling of the metal takes place in the primary cooler, particularly in the nozzle part thereof, the length of which is about 1 - 5 % of the total length of the cooler. The secondary cooling takes place in the top part of the primary cooler and in a separate secondary cooler, which again constitutes about half of the total length of the cooler. The top part of the primary cooler and the secondary cooler comprise an outer shell, a cooling water distribution pipe and an inner pipe. The cooling water is outside the inner pipe and the wire to be cast is inside. In between the inner pipe and the wire to be cast, there must be arranged a clearing in order to allow the billet to move without obstacle. Heat transfer takes place over the gap between the wire to be cast and the inner pipe.

In the conventional vertical casting process, the relatively high costs of the production line are a remarkable factor, particularly when talking about a limited production, because the structures must be provided in the same fashion as in production lines with a larger production. The costs of the production line could be lowered by increasing the casting rate, in which case the number of coilers and coolers would be reduced. However, the inefficiency of the secondary cooling forms an obstacle for increasing the casting rate. When the billet is too hot when coming out of the cooler, it is oxidized on the surface and blackened, whereafter it is not accepted for further refining. The maximum casting rate for instance for an unoxidized cast wire with a diameter of 8 mm is about 5m/min when the cooler is clean, the cooling water is sufficiently cold and the melt quality acceptable. Among the obstacles for improving secondary cooling let us point out that the inner pipe cannot be made too tight, because the billet must be able to move freely, and on the other hand it is not profitable to make the coolers much longer owing to the fairly small diameter of the cast wire. A long and thin wire easily looses the impact form made by the casting machine, which has a significant effect to the wire quality.

JP-A 581 87 243 shows a casting nozzle which is integrated in a cover plate covering the surface of the melt. The disadvantage of this known apparatus is the need of a complicated control mechanism for keeping the melt surface at a certain level. JP-A 59 223 144 describes a typical horizontal casting apparatus where a diverting element is provided between the horizontal side outlet of the furnace in the inlet channel of the casting nozzle. This apparatus cannot be used in an upward casting process where a casting nozzle together with a primary cooler is immersed at least partly into the open surface of the melt.

Typical vertical casting nozzles for upward casting are shown in US 3,746,077 and EP 481 380 A1. The documents show casting nozzles with an integrated primary cooler effecting the solidification of the incoming melt and thus the forming of the product to be cast.

The method and apparatus of the present invention is developed particularly for small-capacity needs. In this method the product to be cast - wire, bar or tube - is cast, instead of the conventional vertically upward casting method, upwardly in an inclined position, at an angle of 20 - 85°, advantageously 30 - 60° in relation to the vertical axis of the furnace, and there is provided only one cooler per wire, while the secondary cooling is carried out directly on the piece to be cast. The invention also relates to the respective apparatus. The essential novel features of the invention are apparent from the appended claims.

According to the method of the present invention, the casting nozzle and the cooler are immersed in the melt in an inclined position, so that water sprayed on the cast product and meant for secondary cooling can be poured on the hot, cast product outside the walls of the casting furnace. Moreover, the wire coming out of the cooler need not be much bent to the direction of the coiler.

Thus the apparatus according to the invention employs a short cooler, which in practice means that the cooler only comprises a primary cooler used in conventional vertical casting. The purpose of the short cooler is only to cool the smelting heat off the cast metal and to perform a slight primary cooling in order to obtain solidity in the cast product. On top of the hot cast product emerging from the cooler, there is sprayed water in order to achieve secondary cooling and to drop the product temperature sufficiently low, so that oxidation does not take place anymore. In the upper part of the primary cooler, in the orifice thereof, there is prior to the secondary cooling conducted some suitable protecting gas, such as for instance nitrogen, in order to prevent oxidation.

The apparatus according to the invention is further described with reference to the appended drawing 1, which in cross-section illustrates the operation principles of the apparatus.

The casting apparatus according to figure 1 first of all contains a smelting and casting furnace 1, as well as its support structures 2. The primary cooler 4 and the casting nozzle 3 partly inserted therein are immersed in an inclined position, in the case of the drawing at an angle of about 45°, to the melt contained in the furnace. The melt is solidified inside the casting nozzle, so that the formed wire or bar 5 can be pulled, by means of transmission drums 6, over the bending drum 7. The secondary cooling part of the cast product comprises water jets 8 and a chute 9 placed underneath the cast product and the bending drum in order to recover the water sprayed from the jets. It is also seen in the drawing that along the distance in between the upper orifice 10 of the primary cooler and the secondary cooling part, there is conducted a protective gas screen in order to prevent oxidation. The inclined position of the nozzle enables the use of direct water jets outside the walls of the casting furnace.

As is seen in the drawing, the now developed structure is simple and low, wherefore the process is easily controlled. When there is employed, according to the invention, only one cooler surrounding the cast product, the height of the cooler structure remains only about at a fourth part of the height of a conventional cooler. Moreover, direct water cooling is very efficient, and as a consequence casting speed can be increased higher than in conventional methods without oxidizing the cast product. This in turn results in that the number of the coolers and coilers can be reduced and expenses cut.

In the primary cooler of the now developed apparatus, only about 60 % of the heat amount of the cast product is recovered, which means that the quantity of the required cold water is reduced by about 40 %. The final cooling is carried out by the spray water through direct jets, and it is not subjected to similar high purity and temperature requirements as the water in the primary cooler.

Particularly in small-production casting machines, each cast product has a specific running motor, in which case there are no obstacles for individual starting of each cast product by reducing speed. On the other hand, because every cast product has its own running motor, the size of the motor can be chosen to be very small in order to lower expenses. When the material to be smelted is fed into the casting furnace in an even fashion and the immersion depth of the nozzle is sufficient, a separate height adjusting system that causes expenses can also be left out of the casting machine.

## Claims

1. A method for casting non-ferrous metal wires, bars and tubes comprising following steps:
Immersing a casting nozzle and a primary cooler in the free surface of a melt comprised in a melting furnace at an angle of 20 to 85° with respect to the vertical furnace axis, so that the melt solidifies therein and the formed cast product can be pulled by means of transmission drums,
after having passed the primary cooler the cast product is subjected to a secondary cooling where water jets are directly sprayed onto the cast product.

2. A method according to claim 1
**characterized in**
**that** the casting takes place upwardly at an angle of 30 to 60°.

3. A method according to claim 1 or 2,
**characterized in**
**that** the cast product is surrounded by a protective gas in the area between the primary cooling zone and the secondary cooling part.

4. An apparatus for casting non-ferrous wires, bars or tubes (5) in an upwardly direction, said apparatus comprising a smelting and casting furnace (1) comprising a melt with a free smelting surface therein,
and a casting nozzle (3) and a primary cooler (4), whereby the casting nozzle being arranged partly inside the primary cooler, the casting nozzle and the primary cooler being designed to be immersed in the free surface of said melt and extending upwards from the furnace at an angle of 20 to 85° with respect to the vertical furnace axis,
transmission drums (6) located behind the nozzle/primary cooler as to pull the cast product formed therein,
whereby in the proceeding direction of the product to be cast in succession to the primary cooler (4) a secondary cooling part (8) is provided, which comprises means (8) for spraying water jets directly on the product as well as a chute (9) for recovering the water.

5. An apparatus according to claim 4,
**characterized in**
**that** the casting nozzle and the primary cooler extend upwards from the furnace at an angle of 30 to 60° with respect to the vertical furnace axis.

6. An apparatus according to claim 4 or 5,
**characterized in**
**that** the secondary cooling part is located outside the walls of the casting furnace (1).

7. An apparatus according to any of claims 4 to 6,
**characterized in**
**that** between the upper orifice of the primary cooler and the secondary cooling part a protective gas screen is provided.

## Patentansprüche

1. Verfahren zum Gießen von Nichteisen-Metalldrähten, Stangen und Rohren, welches folgende Schritte umfasst:
Eintauchen eines Gießmundstückes und eines Primärkühlers in die freie Oberfläche einer in einem Schmelzofen enthaltenen Schmelze unter einem Winkel von 20 bis 85° in Bezug auf die vertikale Ofenachse, so dass die Schmelze darin erstarrt und das geformte Gießprodukt mittels Übertragungstrommeln gezogen werden kann, und das Gießprodukt, nachdem es den Primärkühler passiert hat, einer Sekundärkühlung ausgesetzt wird, wo Wasserstrahlen direkt auf das Gießprodukt gesprüht werden.

2. Verfahren nach Anspruch 1,
**dadurch gekennzeichnet, dass** das Gießen von unten nach oben unter einem Winkel von 30 bis 60° stattfindet.

3. Verfahren nach Anspruch 1 oder 2,
**dadurch gekennzeichnet, dass** das Gießprodukt in dem Bereich zwischen der Primärkühlzone und dem Sekundärkühlteil von einem Schutzgas umgeben ist.

4. Vorrichtung zum Gießen von Nichteisen-Metalldrähten, Stangen oder Rohren (5) von unten nach oben, welche Vorrichtung einen Schmelz- und Gussofen (1) umfasst, welcher eine Schmelze mit einer freien Schmelzoberfläche enthält, und ein Gießmundstück (3) und einen Primärkühler (4), wobei das Gießmundstück zum Teil in dem Primärkühler angeordnet ist und das Gießmundstück und der Primärkühler so konstruiert sind, dass sie in die freie Oberfläche der Schmelze eintauchen und sich unter einem Winkel von 20 bis 85° in Bezug auf die vertikale Ofenachse nach oben aus dem Ofen erstrecken, und hinter dem Mundstück/Primärkühler angeordnete Übertragungstrommeln (6) umfasst, um das darin geformte Gießprodukt zu ziehen, wobei in der laufenden Richtung des zu gießenden Produktes auf den Primärkühler (4) folgend ein Sekundärkühlteil (8) vorgesehen ist, welches Mittel (8) um Wasserstrahlen direkt auf das Produkt zu sprühen umfasst, als auch eine Rutsche (9) zur Wiederverwendung des Wassers.

5. Vorrichtung nach Anspruch 4,
**dadurch gekennzeichnet, dass** sich das Gießmundstück und der Primärkühler unter einem Winkel von 30 bis 60° in Bezug auf die vertikale Ofenachse nach oben aus dem Ofen erstrecken.

6. Vorrichtung nach Anspruch 4 oder 5,
**dadurch gekennzeichnet, dass** das Sekundärkühlteil außerhalb der Wände des Gießofens (1) angeordnet ist.

7. Vorrichtung nach einem der Ansprüche 4 bis 6,
**dadurch gekennzeichnet, dass** zwischen der oberen Mündung des Primärkühlers und dem Sekundärkühlteil eine Schutzgasabschirmung vorgesehen ist.

## Revendications

1. Procédé pour la coulée de fils métalliques non-ferreux, de barres et de tubes comprenant les étapes suivantes :
La plongée d'une buse de coulée et d'un premier dispositif de refroidissement dans la surface libre d'une fonte située dans un four de fonte dans un angle de 25 à 85° par rapport à l'axe vertical du four de sorte que la fonte se solidifie à l'intérieur et que le produit coulé formé puisse être tiré aux moyens de tambours de transmission.
Après avoir subi le premier refroidissement, le produit coulé est l'objet d'un deuxième refroidissement pendant lequel les jets d'eau sont directement dispersés sur le produit coulé.

2. Procédé selon la revendication 1 **caractérisé en ce que** la coulée a lieu vers le haut à un angle compris entre 30 et 60°.

3. Procédé selon la revendication 1 ou 2 **caractérisé en ce que** le produit coulé est entouré d'un gaz protecteur à l'endroit situé entre la zone du premier refroidissement et la partie du deuxième refroidissement.

4. Procédé pour la coulée de tubes non-ferreux, de barres ou de tubes (5) dans une direction vers le haut ; ledit procédé comprenant un four de fonte et de coulée (1) contenant une fonte avec une surface de fonte libre à l'intérieur, une buse de coulée (3) et un premier dispositif de refroidissement (4), dans lequel procédé la buse de coulée est disposée en partie à l'intérieur du dispositif de refroidissement ; la busée de coulée et le premier dispositif de refroidissement étant destinés à être plongés dans une surface libre de ladite fonte et s'étendant vers le haut à partir d'un angle compris entre 20 et 85° par rapport à l'axe vertical de four, comprenant des tambours de transmission (6) situés derrière la buse/le premier dispositif de refroidissement afin de tirer le produit coulé s'y étant formé, alors que dans la direction d'exécution du produit à couler, on fournit une deuxième partie de refroidissement pour faire suite au premier dispositif de refroidissement comprenant des moyens (8) pour disperser des jets d'eau directement sur le produit ainsi qu'une rainure (9) pour récupérer l'eau.

5. Dispositif selon la revendication 4, **caractérisé en ce que** la buse de coulée et le premier dispositif de refroidissement s'étendent vers le haut à partir du four dans un angle compris entre 30 à 60° par rapport à l'axe vertical du four.

6. Dispositif selon la revendication 4 ou 5, **caractérisé en ce que** la partie du deuxième refroidissement est située hors des parois du four de coulée (1).

7. Dispositif selon une quelconque des revendications 4 à 6, **caractérisé en ce qu'**entre l'orifice supérieur du premier dispositif de refroidissement et la deuxième partie de refroidissement, il est fourni un écran de gaz.
